

## UNITED STATES PATENT OFFICE

2,122,940

## LUBRICANT

Walter D. Hodson, Chicago, Ill.

No Drawing. Application December 17, 1934,  
Serial No. 757,969

16 Claims. (Cl. 87—9)

The present invention relates to improvements in greases, and will be fully understood from the following description thereof.

This application is a continuation-in-part of my copending application Serial Number 412,929.

The present invention relates to greases of an unctuous character consisting principally of a lubricant oil and a gelling metallic soap, such greases having a great adherence to the parts to be lubricated and a strong resistance to being squeezed out under load. Ordinarily lead soaps are employed in such greases, such as the lead soaps of oleic acid, fish oils, stearic acid, castor oil, linseed oil, degras, rosin, or naphthenic acids. Other gelling metallic soaps which may be employed are the similar soaps of aluminum, calcium, zinc, copper, manganese, magnesium and the like. In general, the use of the lead soaps, for example, the naphthenate, oleate or fish oil soaps, is preferred. However, soaps of other metals or mixtures of soaps of different metals or other gelling or body-imparting materials capable of imparting to the oil the desired characteristics may be employed. Water-soluble soaps such as sodium soaps may be used, but with such soaps, particular care must be used to prevent the formation of soluble oils such as cutting oil.

In the manufacture of such greases, wherein adhesion and resistance to squeezing out under load are desired, it is necessary to incorporate into the mineral lubricant oil employed substantial quantities of the non-setting, gelling soap. For example, the proportions desired may be as high as from 20% to 60% of the soap, but such proportions of the soap result in an extremely heavy, viscous material which does not readily flow and the use of which may be entirely impractical in bearings with small clearance or when there is occasional or continuous exposure to a low temperature. The low fluidity of such greases has rendered necessary the use of relatively small proportions of the soap, or has prevented entirely the use of such compounds.

I have found that a fluidity of such compounds may be modified by incorporating therein a small proportion, ranging ordinarily from  $\frac{1}{2}\%$  to 10%, of organic oil-miscible solvents having a boiling point of  $80^{\circ}$  C. or higher, and preferably of from 150 to  $250^{\circ}$  C. These organic solvents, which are completely miscible with the oil-soap compound, are of the type now generally designated as lacquer solvents. For example, I have successfully employed such oil-miscible solvents as ethylene dichloride, dichlorethylether, diethyleneglycol, the monoalkylethers of ethyleneglycol and diethyleneglycol and their esters, such as ethyleneglycol, monoethylether, ethyleneglycol, monoethylether acetate, ethyleneglycol monobutylether, diethyleneglycol monoethylether, diethyl-

ene glycol monobutylether, triethanolamine, and the like. Equivalent solvents such as phenyl chlorides, including monochlor benzene, ortho-dichlor benzene, and trichlor benzene may likewise be used. The phenyl chlorides, and particularly monochlor benzene are preferred for calcium base greases. For example, I have found ethyleneglycol monoethylether, dichlorethylether, and ethylene dichloride to be particularly desirable in increasing the fluidity of such compounds. The proportion of such solvents which may be employed varies, depending upon the characteristics of the compound in which it is incorporated and the characteristics desired in the final product. Thus, from  $\frac{1}{2}$  to 1% of the solvent has an appreciable effect in reducing the viscosity and increasing the fluidity of the compound. Ordinarily, for example, with a content of lead fish oil soap, say of 5 to 30%, from 3 to 5% of such a solvent, for example, dichlorethylether or ethylenedichloride may be employed. With the compounds containing higher proportions of the soap, say 30 to 60%, up to 10% or even more of the solvent may be incorporated. The solvent may be selected and the proportions thereof adjusted in accordance with the desired use. For example, in bearings with smaller clearances, more solvent may be employed to secure a greater fluidity, and a more volatile solvent may be employed to permit its rapid evaporation.

Occasionally, the compounds containing the solvent may show some settling on long standing, as in compounds containing a small amount of the soap in a low-viscosity oil and I have found that this may be prevented by incorporating into the composition a small proportion of a high boiling organic ester, having preferably a boiling point of from 250 to  $450^{\circ}$  C. or higher. For example, I have employed for this purpose such esters as tricresyl phosphate, butyl phthalate, amyl phthalate, dibutyl phthalate, butyl stearate, ethyl acetate, or the like. Dibutyl phthalate I have found to be particularly effective. From  $\frac{1}{2}$  to 2 or 5% of such high boiling esters, while miscible with the oil and the oil solvent employed, are ordinarily sufficient.

As will be readily understood, the lubricant oil employed and the specific metallic soap will be selected in accordance with the practice of the art to secure the desired type of lubrication. Thus, for small high speed units, the gears and bearings require a relatively low viscosity mineral oil, say 75 to 150 sec. Saybolt at  $100^{\circ}$  F., while for heavier duty gears and bearings, higher viscosity oils may be employed and larger proportions of the soap may be present. The presence of the solvent and the stabilizing material in accordance with the present invention does not materially alter the lubricating characteristics of the compound apart from markedly in-

creasing its fluidity and extending its adaptability in use. The compound retains its desirable qualities of adherence to metal and resistance to squeezing out under load. The solvent 5 may be in part dissipated in use, but since such loss occurs after application of the lubricating compound, and after its penetration into the working parts of the bearing or gearing, it does not adversely affect the value of the compound, 10 but is, in fact, frequently desirable.

A sodium soap grease may be prepared containing 10-50% of a sodium soap such as oleate, stearate or the like (preferably tallow fat acids) and the balance mineral oil of the desired viscosity. A typical grease will contain 30% sodium soap and 70% of a heavy steam-refined cylinder stock mineral oil, for example, having a viscosity of 200° Saybolt at 210° F. Such a grease will be extremely hard, and particularly suitable for use 15 in lubricating roll neck bearings. With the particular sodium soap described 2½% of butyl Carbitol is preferred as a solvent.

The foregoing detailed description has been given for clearness of understanding only, and 20 no unnecessary limitations should be understood therefrom, but the appended claims should be construed as broadly as permissible in view of the prior art.

What I claim as new and desire to secure by 25 Letters Patent is:

1. An adherent, fluid, lubricating compound composed principally of a viscous mineral oil and a non-setting, gelling soap, said compound including a minor proportion of an aliphatic oil-miscible grease-compatible organic solvent whereby the fluidity thereof is increased, and a stabilizing organic ester, selected from a group 35 consisting of tricresyl phosphate, butyl phthalate, amyl phthalate, dibutyl phthalate, butyl stearate, and ethyl acetate.

2. An adherent, fluid, lubricating compound composed principally of a viscous mineral oil and a non-setting, gelling soap, said compound including a minor proportion of an aliphatic oil-miscible grease-compatible organic solvent, 45 whereby the fluidity thereof is increased, and a stabilizing organic ester having a boiling point between 250° and 450° C., selected from a group comprising tricresyl phosphate, butyl phthalate, amyl phthalate, dibutyl phthalate, butyl stearate, and ethyl acetate.

3. An adherent, lubricating compound composed principally of a viscous mineral oil and a non-setting, gelling soap, said compound including a minor proportion of an oil-miscible grease-compatible organic solvent containing a monoalkyl-glycolether group, whereby the fluidity 55 thereof is increased, and a high boiling organic ester selected from a group consisting of tricresyl phosphate, butyl phthalate, amyl phthalate, dibutyl phthalate, butyl stearate and ethyl acetate.

4. An adherent, fluid lubricating compound composed principally of a viscous mineral oil and a non-setting gelling soap, said compound including dichlorethylether in quantity sufficient 65 to increase the fluidity thereof.

5. An adherent, fluid lubricating compound composed principally of a viscous mineral oil and a non-setting, gelling soap, said compound including diethylene glycol monobutyl ether in 70 quantity sufficient to increase the fluidity thereof.

6. An adherent, fluid lubricating compound composed principally of a viscous mineral oil and a non-setting, gelling soap, said compound including ethylene dichloride in quantity sufficient to increase the fluidity thereof. 5

7. An adherent, fluid lubricating compound composed principally of viscous mineral oil and a non-setting, gelling soap, said compound including a minor proportion of ethylene dichloride and a small proportion of dibutyl phthalate. 10

8. An adherent, lubricating compound containing a mineral oil, from 10 to 30% of a lead soap, and from 3 to 5% of an oil-miscible grease compatible hydrocarbon derivative solvent capable of increasing the fluidity thereof 15 without materially affecting the lubricating properties of the lubricating compound.

9. An adherent, lubricating compound composed of a viscous mineral oil and from 10 to 30% of a lead soap, said compound including from 3 to 5% of an aliphatic oil-miscible grease-compatible organic solvent and from ½ to 3% of a high boiling point ester, selected from a group consisting of tricresyl phosphate, butyl phthalate, amyl phthalate, dibutyl phthalate, 25 butyl stearate and ethyl acetate.

10. A method of modifying the fluidity of greases composed principally of viscous mineral oil and a metallic soap, said soap being present in an amount sufficient to produce a grease structure 30 of the character produced in a lead soap by the presence of approximately 5-30% of the lead soap, which consists in adding an oil-miscible solvent of the class consisting of ethylenedichloride, dichlorethylether, diethyleneglycol, the monoalkyl ethers of the ethyleneglycol and diethyleneglycol and their esters and phenyl chlorides. 35

11. An adherent fluid grease composed principally of a viscous mineral oil and a metallic soap, the soap being present in an amount sufficient to 40 produce a solid grease structure, and said compound including a minor proportion of an oil-miscible organic solvent of the class consisting of ethylenedichloride, dichlorethylether, diethyleneglycol, the monoalkyl ethers of ethyleneglycol and 45 diethyleneglycol and their esters, and phenyl chlorides, whereby the grease is rendered fluid without material impairment of its grease characteristics.

12. An adherent fluid grease composed principally of a viscous mineral oil and a gelling metallic soap, the soap being present in that amount sufficient normally to produce a grease solid at 50 normal temperatures and said grease compound including a small proportion of a liquid oil-miscible, grease-compatible, hydrocarbon derivative organic solvent, whereby the fluidity thereof is markedly modified without materially affecting the lubricating faculties of the grease compound.

13. A grease as set forth in claim 12, in which 55 the organic solvent has a boiling point from 80° C. to 250° C.

14. A compound as set forth in claim 12, in which the organic solvent is present in an amount from ½ to 10% of the grease. 65

15. A compound as set forth in claim 12, in which the solvent contains a monoalkylglycol-ether group. 70

16. A compound as set forth in claim 12, in which the organic solvent is diethyleneglycol-monobutylether.

WALTER D. HODSON.